

S. B. NEWBERRY & H. N. BARRETT.  
PROCESS OF MAKING PHOSPHATE FERTILIZERS.  
APPLICATION FILED NOV. 4, 1912.

1,162,944.

Patented Dec. 7, 1915.



Witnesses.

Edward T. Gray.

Minnie M. Lindenau

Inventors.  
Spencer B. Newberry.  
Harvey N. Barrett.  
by Parker & Carter  
Attorneys.

# UNITED STATES PATENT OFFICE.

SPENCER B. NEWBERRY AND HARVEY N. BARRETT, OF BAYBRIDGE, OHIO.

## PROCESS OF MAKING PHOSPHATE FERTILIZERS.

1,162,944.

Specification of Letters Patent.

Patented Dec. 7, 1915.

Application filed November 4, 1912. Serial No. 729,299.

To all whom it may concern:

Be it known that we, SPENCER B. NEWBERRY and HARVEY N. BARRETT, citizens of the United States, residing at Baybridge, in 5 the county of Erie and State of Ohio, have invented a certain new and useful Improvement in Processes of Making Phosphate Fertilizers, of which the following is a specification.

10 This invention relates to improvements in the process of rendering natural phosphates available for use as fertilizers.

15 The particular apparatus whereby the invention can be carried out is illustrated in the accompanying drawings, in which—

Figure 1 is a side elevation of the kiln and Fig. 2 is a section on line 2—2 of Fig. 1.

20 The kiln A rests upon rollers B B and is revolved by gearing not shown in the drawing. It is heated internally by a flame or flames of coal-dust, oil or gas, blown in with air through G. The phosphate mixture is introduced into the space I, in which, if wet, it is rapidly dried by the hot gases

25 and by contact with the hot lining. The dried mixture passes down the kiln, being lifted and turned over by the shelves F F, and is kept from reaching too high temperature by radiation of heat through the lining E. Between the drying zone I and the middle point of the kiln the mixture is exposed to moderate temperature, and from the middle point to the lower end of the shelves it is subjected to the highest heat.

30 35 The calcined product is discharged through the hood H into the cylinder C, in which it is cooled by air drawn in by the draft of the stack.

In order that the process may be fully 40 understood, we will describe it more or less in detail, and particularly set forth those details of operation which, when closely followed, are likely to give the best and most economical results, having reference to the 45 process of calcination of phosphates with the addition of a small percentage of reagents, as for example, alkalis or alkali-metal salts. These details of operation are as follows:

50 1. The conversion to citrate-soluble con-

dition is brought about by exposure of the phosphate to sufficiently prolonged and intimate contact with a rapid current of highly heated gases. To produce and maintain this intimate contact it is most important 55 that the material treated shall be in a porous and cellular condition, in order that the gases may penetrate and envelop every particle or portion of the substance. This we accomplish by grinding the phosphate to a 60 liquid slurry and introducing this slurry at the upper end of the revolving kiln in which the calcining is effected.

We wish it to be understood that we do not limit ourselves to the above-described 65 method of securing a porous cellular or laminated condition of the phosphate mixture, and that other devices or manipulations by which free circulation of the hot gases through all parts of the material 70 treated may be secured do not constitute a departure from our process as herein set forth.

2. If the phosphate in admixture with alkali-metal compounds is heated while at 75 rest or out of intimate contact with the hot gases, it tends to fuse together into compact grains or lumps, which in the further process of calcination are scarcely at all converted into citrate-soluble form. To 80 avoid this injurious effect it is necessary that the material during the whole course of the heating shall be actively agitated and turned over, thus thoroughly promoting continued contact of the gases with every part of the 85 charge and preventing the formation of lumps which would escape further action. This agitation is effected by the revolution of the kiln and increased by the lifting and rolling action of a number of shelves or 90 ridges in the kiln lining, which extend from the end of the drying zone nearly to the point of discharge of the calcination product.

3. In the first stage of the heating the 95 temperature of the charge increases rapidly, and under the combined action of heat, agitation and intimate contact with a rapid current of hot gases the alkali-metal compound is rapidly decomposed with evolution 100

of its acid or other volatile constituents. This action takes place actively at a temperature of 2000 degrees F. or over, provided the material is porous and the current of hot gases sufficiently rapid. Under these conditions such alkali-metal compounds as hydrate, sulfate or carbonate, which are scarcely affected by heating to much higher temperatures when at rest, are rapidly decomposed with evolution, respectively, of water, sulfur dioxid and oxygen, and carbon dioxid, leaving a residue of alkali-metal oxid which we term "residual alkali." The volatile constituents may be said 15 to be "blown out" of the salts by contact with the current of hot gases. It is probable that the residual alkali enters into combination with the phosphate of lime, forming an alkali-lime phosphate which is again 20 in large measure decomposed at the higher temperature of the later stage of the process, and that this combination and subsequent decomposition plays an important part in the conversion of the phosphate into 25 citrate-soluble condition.

4. In the final stage of calcination a temperature of about 2400 degrees to 2600 degrees F. is required, and in this stage, under the combined action of heat, agitation and 30 intimate contact with a rapid current of highly heated gases, the residual alkali is in turn and in large measure volatilized, and simultaneously with the expulsion of alkali the percentage of citrate-soluble phosphoric 35 acid rapidly increases, until, with proper adjustment of temperature and duration of heating, the conversion to citrate-soluble condition becomes practically complete, only traces of insoluble phosphoric acid remaining. The product of the operation conducted as above described appears in the form of brown or black masses or fragments, extremely porous and light, and so soft that it can be crushed to powder by pressure of 40 the fingers. During the entire course of the calcination the expulsion of the volatile constituents of the alkali-metal compound and of the residual alkali tends to prevent over-heating and fusion of the material. 45 This expulsion takes place normally and rapidly if the material is exposed to and penetrated by a rapidly-moving current of hot gases, for example such a current as is produced by introducing the fuel at the 50 lower end of the kiln in admixture with a current of air under four or five ounces pressure and by maintaining a strong draft in the stack at the upper end of the kiln. Under these conditions the material remains 55 in a porous and light condition throughout its passage through the kiln, the volatile constituents of the alkali-metal salt are completely expelled in the zone of moderate heat, the residual alkali is chiefly expelled 60

in the final stage of heating, and the phosphate is rendered practically completely citrate-soluble. On the other hand, if the current of hot gases is slow and sluggish or does not freely penetrate the charge, little or no decomposition and expulsion of the 65 alkali-metal salt takes place, the material fuses or sinters together into impervious masses, and practically no conversion into citrate-soluble condition is effected.

An additional safeguard against the fusion or agglomeration of the material, especially in the earlier stage of heating, consists in carrying on the calcination in a kiln provided with a comparatively thin refractory lining, through which radiation of heat 75 takes place to a considerable degree. The effect of this radiation is to keep the interior of the kiln walls at a somewhat lower temperature than that of the charge or the gases passing through the apparatus, and 80 thus to prevent the charge from becoming over-heated and fused by contact with the 85 hot lining.

By "alkali-metal compound" we mean any compound of the alkali-metals as potassium 90 or sodium, with hydroxyl or the common acids, for example the hydrate, carbonate, chlorid, sulfate, bisulfate, nitrate, etc. We prefer to use sodium sulfate or bisulfate, on account of the cheapness of these reagents 95 and the ease with which they undergo decomposition under the conditions of calcination herein described. We find, however, that any compound or combination of the alkali-metals substantially free from ingredients injurious to the process or product 100 produces a result similar to that obtained by the use of the alkali-metal salts above mentioned.

The amount of alkali-metal compound required varies with the nature of the phosphate treated and the temperature employed. Taking sodium sulfate as an example, the addition of 10 to 20 per cent. is sufficient to accelerate and complete the 110 transformation of the phosphate to citrate-soluble condition.

By "volatile constituents" of alkali-metal compounds we mean such part thereof as may be driven off by the action of hot gases 115 under the conditions herein described, leaving a residue of alkali-metal oxid, as for example, water, sulfur dioxid and oxygen, carbon dioxid, oxids of nitrogen, etc. By "residual alkali" we mean the residue, consisting chiefly of alkali-metal oxid, remaining after the expulsion of the volatile constituents of alkali-metal compounds.

By "increasing temperature" we mean a temperature of the material below that of fusion increasing from approximately 2000 degrees F. to 2500 degrees F. By "high temperature" we mean a temperature below 125

the fusing point of the partially calcined phosphate, approximately 2500 degrees F. It is to be understood that higher temperatures than the above are not injurious provided the material is not fused or balled together in such manner as to interfere with the transformation desired.

A suitable kiln for the treatment of phosphate mixtures as herein described consists of a steel cylinder of relatively large diameter and short length as compared with the kilns used in cement burning. For example, a length of from 30 to 50 feet and a diameter of 8 to 10 feet are appropriate relative dimensions. The kiln rests upon rollers and is revolved by power in the usual manner, at a speed of approximately 1 revolution per minute. The inclination of the kiln is relatively considerable, preferably  $\frac{3}{4}$  inch to 1 inch per foot of length. It will be understood, however, that since increased speed and increased inclination produce a similar effect on the movement of the charge, the above figures may be varied considerably. The interior of the kiln is lined with a layer of refractory material, preferably consisting of fire-brick in the upper portion and cement clinker or magnesite brick in the lower part. This lining is provided with a number of low shelves or ridges, extending lengthwise of the kiln, preferably beginning at about one-fourth the length from the upper end and extending nearly to the discharge end of the kiln; the purpose of these ridges is to turn the charge over and prevent it from sliding on the inner surface, and thus to promote exposure of the material to intimate contact with the rapidly moving hot gases. The kiln is heated internally by a flame or flames of coal-dust, oil or gas, and the heat so regulated that a moderately high temperature extends the entire length of the interior. The heat of the gases discharged from the kiln may be utilized in boilers or for other purposes, by well-known methods. Suitable devices for cooling the discharged product by a current of air and utilizing the air so heated to support combustion of the fuel may be employed with advantage. We wish it to be understood, however, that we do not limit our invention to the use of a revolving kiln as above described, or to any special form of apparatus, as the process herein set forth may be successfully carried on in any type of kiln or furnace in which the required temperature and free circulation of hot gases through the material are secured.

We claim:

1. The process of making fertilizer by pulverizing natural phosphate of lime, mixing the phosphate with alkali-metal compound, and calcining the mixture in contact with a rapid current of hot gases while agi-

tating to present renewed surfaces to heat, 65 at increasing temperature until the alkali-metal compound is substantially decomposed with evolution of volatile constituents, and finally at high temperature until the phosphate becomes substantially citrate-soluble. 70

2. The process of making fertilizer by pulverizing natural phosphate of lime, mixing the phosphate with alkali-metal compound and calcining the mixture in contact with a rapid current of hot gases while agitating to 75 present renewed surfaces to heat at increasing temperature until the alkali-metal compound is substantially decomposed with evolution of volatile constituents, and finally at high temperature until the residual alkali is 80 partly expelled and the phosphate becomes substantially citrate-soluble.

3. The process of making fertilizer by pulverizing natural phosphate of lime, mixing the phosphate with alkali-metal compound and calcining the mixture in contact with a current of hot gases of such velocity and temperature that volatile constituents of the alkali-metal salt and part of the residual alkali shall be expelled and the material prevented from fusing and kept in a porous condition, at increasing temperature and finally at high temperature until the phosphate becomes substantially citrate-soluble. 85 90 95

4. The process of making fertilizer by pulverizing natural phosphate of lime, mixing the phosphate with alkali-metal compound and water, drying the mixture rapidly in such manner that it shall take a porous cellular form, and calcining the dried porous mixture in contact with a rapid current of hot gases while agitating to present renewed surfaces to heat, at increasing temperature and finally at high temperature 100 105 until the phosphate becomes substantially citrate-soluble.

5. The process of making fertilizer by pulverizing natural phosphate of lime, mixing the phosphate with alkali-metal compound and water, drying the mixture rapidly in such manner that it shall take a porous cellular form, and calcining the dried porous mixture in contact with a rapid current of hot gases while agitating to present 110 renewed surfaces to heat, at increasing temperature until the alkali-metal compound is substantially decomposed with evolution of volatile constituents and finally at high temperature 115 until the residual alkali is partly 120 expelled and the phosphate becomes substantially citrate-soluble.

6. The process of making fertilizers by pulverizing natural phosphate of lime, mixing the phosphate with alkali-metal compound, preparing the mixture in such manner as to give it a porous and open structure, freely permeable by gases, and calcining the 125

prepared mixture in contact with a rapid current of hot gases, at increasing temperature until the alkali-metal compound is substantially decomposed with evolution of volatile constituents and, finally at high temperature until the residual alkali is partly expelled and the phosphate becomes substantially citrate soluble.

Signed at Sandusky, Ohio, this thirty-first day of October, 1912.

SPENCER B. NEWBERRY.  
HARVEY N. BARRETT.

Witnesses:

HATTIE M. MEGGITT,  
ALLEN KUBACH.